

## UNITED STATES PATENT OFFICE

2,598,854

## ASBESTOS-ALUMINUM POWDER PAINT

Frederick A. Stolz, San Francisco, and Edley J. Vaught, Jr., Oakland, Calif., assignors to Pabco Products Inc., a corporation of Delaware

No Drawing. Application July 22, 1950,  
Serial No. 175,468

6 Claims. (Cl. 260—28.5)

**1**  
This invention relates to a metallic bituminous paint, and more particularly to such paint containing flaked aluminum powder which imparts to the dry paint coating or film an ornamental metallic appearance, and which also contains a filler the majority of which is asbestos fiber to enable the paint to be applied as a single relatively thick coat compared to such paint without the filler.

A paint of this character is disclosed in assignee's patent to Buchanan, No. 2,477,236, dated July 26, 1949, in which the binder for the paint is entirely of bituminous material, and the paint is solvent-thinned so that its viscosity is such as to enable it to be applied to a surface by brushing or spraying.

Summarizing this invention, the paint thereof is an improvement over the paint disclosed in the patent, by increase of the solvent content of the paint with respect to the quantity of binder in the paint, so that the aluminum powder or flakes will have enhanced floating power to the surface of the paint when applied and thus provide an improved metallic color and retention of such color at the surface, and also increase of the filler content of the paint compared to the quantity of the binder to improve the matting qualities of the paint.

In addition, instead of a binder which is entirely of bituminous material as is disclosed in the patent, the binder of this invention is a mixture of bituminous material and a relatively light colored resin derived from coal tar (hereinafter referred to as coal tar derivative resin), preferably a coumarone-indene resin well known in the varnish making art. Such resin is compatible with the bituminous material of the binder. The invention has as its objects, among others, the provision of an improved paint of the character related, having enhanced floatability of the aluminum powder and an improved binder in the paint, which is economical and easy to apply by brushing or by spraying, and which can be readily manufactured.

The improved binder of the paint is an important feature of the invention because if the binder is entirely of bituminous material, such as asphalt, as disclosed in the aforementioned patent, it sometimes turns brown after exposure to the elements for a substantial period of time and discolors the aluminum flakes or powder which may have worked up to the surface of the paint. Incorporation of the light colored coal tar derivative resin in the bituminous material of the binder obviates this problem and

**2**  
preserves the brilliancy of the metallic film. In this connection, petroleum derivative resins are not satisfactory for this purpose. Although any suitable relatively light colored coal tar derivative resin common in the varnish making art may be utilized, coumarone-indene resins employed in the varnish making art, are most satisfactory, and the coumarone-indene resin known in the trade as "EX Cumar" is preferred. This resin has a melting point in the range of 100° C. to 115° C., and is substantially non-acid, having a substantially neutral reaction.

About equal proportions by weight of the resin and the bituminous material provide the most satisfactory binder and are preferred. If too much resin is employed, cracking or so-called "alligatoring" of the dried binder film may result. Too little of the resin will not overcome the discoloration effect previously mentioned. About the maximum amount of resin that should be utilized is 75 parts by weight to about 25 parts by weight of the bituminous material. The minimum amount is about 25 parts by weight of the resin to about 75 parts by weight of the bituminous material. Thus, the binder has the following formulation range.

|    | Percent and Parts by Weight |     |
|----|-----------------------------|-----|
| 30 | Bituminous material.....    | 75  |
|    | Resin.....                  | 25  |
|    | Total.....                  | 100 |
|    |                             | 75  |
|    |                             | 25  |
|    |                             | 100 |

35 The bituminous material is required in the binder in order to render the paint compatible with the usual bituminous coating on felt base roofing material for which the paint is particularly adapted as a coating therefor.

40 The paint consists essentially of the described binder, volatile solvent for the binder, filler which is preferably all asbestos fiber, but if not, the majority of which is asbestos fiber, and the flaked aluminum powder. In other words, substantially all or 100% of the paint is composed of these four materials. The volatile solvent is the major constituent in that the quantity by weight is in excess of any other substance of the paint, and is in such excess with respect to the weight of the aluminum powder and the weight of the binder as to cause the powder to float to the surface of the fresh paint without being covered by a substantial film of the binder.

45 According to the improved range of proportions of the instant formulation, the total quan-

tity of binder and the solvent constitutes from about 67% to about 82% by weight of the total weight of the paint, and the total quantity of the filler and the aluminum powder about 18% to about 33% of the total weight of the paint. Although the ratio of the aluminum powder to the filler is not so critical to obtain the improved metallic appearance of the paint, the solvent to binder ratio should be from about 3 to 6 parts by weight of the solvent to about 1 part by weight of the binder. The amount by weight of the filler to the aluminum powder may vary from about 0.8 to 2.5 parts by weight of the filler to about 1 part by weight of the powder.

Preferably, the amount by weight of the aluminum powder to the binder should be somewhat less than that of the binder but may vary from about 1 to about 2 parts by weight of the binder to about 1 part by weight of the aluminum powder. The amount by weight of the filler to the binder may vary from about 0.55 to 1.7 parts by weight of the binder to about 1 part by weight of the filler, but it is desirable that the filler be in excess with respect to the binder for best matting effect.

The following formula expresses the preferred range of proportion in approximate parts and percent by weight.

|                                                                                                                                      | Percent and Parts by Weight |     |
|--------------------------------------------------------------------------------------------------------------------------------------|-----------------------------|-----|
| Binder (composed of mixture of bituminous material and coal tar derivative resin in the range of proportions referred to above)..... | 12                          | 17  |
| Volatile solvent for the binder.....                                                                                                 | 70                          | 50  |
| Aluminum powder.....                                                                                                                 | 8                           | 12  |
| Filler (preferably asbestos fiber).....                                                                                              | 10                          | 21  |
| Total.....                                                                                                                           | 100                         | 100 |

The preferred commercial formulation will be described hereinafter.

As is described in the aforementioned patent, instead of substantially pure aluminum powder, any of the well known commercial aluminum pastes suitable for blending with varnish, or other vehicle for making bronzing paints may be employed instead. Such aluminum paste contains volatile solvent; and when employed, the quantity of volatile solvent otherwise used in a specific paint formula should be reduced a proportionate amount. Aluminum paste contains approximately 30 to 35 percent by weight of volatile solvent; so that with the powder, approximately 30 to 35 percent less by weight is used in the paint compared to the quantity of aluminum paste, and the difference made up by additional solvent.

With respect to the preceding formula range, and subsequent particular formulae, only aluminum powder appears. Consequently, it is to be understood that the proportions of the aluminum and the solvent may be varied along the lines discussed according to whether the aluminum paste is substituted for the aluminum powder, or vice versa. The same is to be understood with respect to claims that recite proportions.

As the filler, asbestos type fiber is the most suitable; and it is preferred for best results. Preferably, the fiber is so-called Canadian asbestos fiber of 0-0-10-6 commercial grade, namely the number of ounces of fiber in a 16 ounce sample that are retained on successive screens of  $\frac{1}{2}$  in.,  $\frac{1}{4}$  in., and  $\frac{1}{8}$  in. mesh and that pass through the  $\frac{1}{16}$  in. mesh, respectively. The coarser the fiber the rougher will be the surface

of the resultant paint coating. This determines the coarseness of the fiber from a practical purpose.

A fiber having a grading of 0-4-8-4 on the same basis mentioned will produce a usable product but in addition to a rougher film, the paint itself will not have as good a spreading capacity as the paint with finer fiber. Finer fiber, as low as 0-0-1-15 grading or even lower, may be employed but then the paint may not result in as thick a film as desired. In place of the preferred Canadian asbestos fiber, other sources of asbestos may be employed, such as Arizona or Vermont asbestos, which lend themselves readily to breaking up into the preferred mesh size and which may be readily dispersed in the paint.

Some of the fiber may be replaced by suitable extenders, such as comminuted diatomaceous earth, powdered talc or soapstone. If diatomaceous earth is employed, about 20% to 30% of the volume of asbestos fiber may be replaced by the earth. Powdered talc or soapstone may be substituted pound for pound for an equal weight of the asbestos fiber, up to about 20% of the total weight of fiber. Finely ground anthophyllite or tremolite may be used under similar conditions. It is important for best results that a substantial proportion or majority of the filler be of the asbestos type fiber, although some of the asbestos type fiber may be replaced in part by suitable extenders.

In addition to extenders of the type described above, color effects may be obtained in the paint by employment of suitable relatively small proportions of color pigments to replace some of the fiber, or extenders if employed, without loss of the metallic appearing surface produced by the aluminum powder. For example, iron oxide may be used to produce a pleasing reddish color almost like metallic copper. Graphite may be used to produce a metallic slate appearance, and chrome oxide will impart a greenish tinge to the metallic lustre created by the aluminum. These pigments are employable in conjunction with the essential ingredients of our paint, namely, the filler, preferably asbestos type fiber, the binder, the aluminum powder, and the volatile solvent.

Asphalt is the preferred bituminous material in the binder; and although asphalt of the specific type disclosed in the aforementioned patent may be employed, it is desirable because of the presence of the resin in the binder, to employ asphalt having a somewhat lower softening point, namely, an asphalt having an A. S. T. M. (Ball and Ring method) softening point in the range of 110° F. to 120° F., and an A. S. T. M. penetration at 77° F. in the range of 51 to 60.

Coal tar pitches having characteristics similar to the preferred asphalt may be used as the bituminous material in the binder. However, "stearine" pitches, although they may be employed, do not produce as good results as the asphalt, or coal tar pitches.

For enhancement of superior floating effect in bringing the aluminum powder to the surface, the volatile solvent should have a high aromatic content such as the crude coal tar naptha solvent disclosed in the aforementioned patent. The floating effect makes for increased brilliancy obtainable by the aluminum powder. Coal tar solvents have the desired high aromatic content, and other coal tar solvents such as toluol and xylol may be employed. The solvent may be en-

tirely of the coal tar type described but because of the presence of the resin in the binder, it lends itself to dilution very readily with the much less costly mineral spirit type of solvents which are well known straight chain olefine hydrocarbons derived from petroleum.

If straight mineral spirits were employed alone as the solvent, the desirable floating effect could not be obtained. Consequently, for obtaining such floating effect, the solvent should have at least 10% by weight of the high aromatic content solvent mentioned, and preferably not less than 20% by weight of such high aromatic content solvent. As previously mentioned, the solvent may be entirely of the high content aromatic type, such as the coal tar solvents, but it is desired to dilute the same in the manner related for purposes of economy.

The preferred coal tar naptha solvent is the same as that described in the patent, having a specific gravity at 15.5° C. in the range of about 0.85 to 0.91, and a distillation temperature in the range of 150° C. to 200° C. The preferred mineral spirit solvent diluent has a specific gravity at 25° F. in the range of 0.79 to 0.82 and a distillation temperature in the range of between 305° F. to 410° F.

The following are typical formulae of the paint of this invention, the formula of Example I being commercially preferred:

*Example I*

|                                                                                                                    | Parts and<br>Percent<br>by Weight | Parts and<br>Percent<br>by Weight |
|--------------------------------------------------------------------------------------------------------------------|-----------------------------------|-----------------------------------|
| Binder                                                                                                             |                                   |                                   |
| Asphalt (A. S. T. M. (Ball and Ring) softening point 110° F. to 120° F. and penetration at 77° F. of 51 to 60)     | 7                                 | 14                                |
| Coumarone-Indene Resin ("EX Cumar") (Melting point 100° C. to 115° C.)                                             | 7                                 |                                   |
| Total                                                                                                              | 14                                | 56                                |
| Volatile Solvent for Binder                                                                                        |                                   |                                   |
| Crude coal tar naptha solvent (Specific gravity at 15.5° C., 0.85 to 0.91) (Distillation range 150° C. to 200° C.) | 13                                |                                   |
| Mineral Spirits (Specific gravity at 25° F., 0.79 to 0.82) (Distillation range 305° F. to 410° F.)                 | 43                                |                                   |
| Total                                                                                                              | 56                                |                                   |
| Aluminum Powder ("Alcoa" A-322)                                                                                    |                                   | 10                                |
| Asbestos Fiber (0-0-10-6 mesh on basis described above)                                                            |                                   | 20                                |
| Total                                                                                                              |                                   | 100                               |

*Example II*

|                                                      | Parts and<br>Percent<br>by Weight | Parts and<br>Percent<br>by Weight |
|------------------------------------------------------|-----------------------------------|-----------------------------------|
| Binder                                               |                                   |                                   |
| Asphalt (same as in Example I)                       | 9                                 | 15                                |
| Coumarone-Indene Resin (Same as in Example I)        | 6                                 |                                   |
| Total                                                | 15                                | 56                                |
| Volatile Solvent for Binder                          |                                   |                                   |
| Crude Coal tar naptha Solvent (Same as in Example I) | 16                                |                                   |
| Mineral Spirits (Same as in Example I)               | 40                                |                                   |
| Total                                                | 56                                |                                   |
| Aluminum Powder (Same as in Example I)               |                                   | 12                                |
| Asbestos Fiber (Same as in Example I)                |                                   | 17                                |
| Total                                                |                                   | 100                               |

Any suitable method may be employed for thoroughly mixing the ingredients to produce a more or less homogeneous mass. A suitable

method of preparation is first to pour a mixture of the bituminous material and the resin in heated molten condition into a suitable heated container, adding the volatile solvent while stirring until a homogeneous mass obtains, cooling to about room temperature after the solvent is thoroughly mixed with the binder, adding the filler while stirring until a uniform mixture is obtained, and finally incorporating the aluminum powder or paste while stirring until all evidence of lumps disappears.

It is possible with the composition of this invention to provide a material which does not have the requisite amount of solvent when packaged, with instructions that it be thinned before use with a specified amount of desired thinner.

However, the paint is preferably employed as a ready-mixed or ready-to-use composition that may be applied directly as a coating, without further mixing, other than the usual mere stirring. The coating formed can be made of the thickness described in the previously mentioned patent. The paint is particularly adapted for application to asphaltic prepared roofing and asphaltic shingles, but it is also useful for the painting of galvanized iron roofing and siding, and for the painting of electric wire and cable. It may be applied either by brush, or by spraying because of its relatively low viscosity.

30 We claim:

1. A solvent thinned metallic ornamental paint consisting essentially of the following in parts by weight:

35 Binder of bituminous material selected from the group consisting of asphalt, coal tar pitches and stearine pitches and coumarone-indene resin in the proportions of about 25% to 75% by weight of bituminous material to about 75% to about 25% by weight of the resin, respectively 12 to 17

40 Volatile solvent for the binder comprising a coal tar solvent 70 to 50

45 Aluminum powder 8 to 12

Filler, the major proportion of which is asbestos fiber 10 to 21

2. A solvent thinned metallic ornamental paint consisting essentially of the following in parts by weight:

55 Binder of asphalt and coumarone-indene resin in the proportions of about 25% to 75% by weight of asphalt to about 75% to about 25% by weight of the resin, respectively 12 to 17

60 Volatile solvent for the binder comprising at least 10% by weight of a coal tar solvent 70 to 50

65 Aluminum powder 8 to 12

Filler, the major proportion of which is asbestos fiber 10 to 21

3. A solvent thinned metallic ornamental paint consisting essentially of the following in parts by weight:

70 Binder of about 50% by weight of coumarone-indene resin and about 50% by weight of asphalt 12 to 17

Volatile solvent for the binder comprising at least 20% by weight of a coal tar solvent 70 to 50

75 Aluminum powder 8 to 12

Filler, the major proportion of which is asbestos fiber 10 to 21

4. A solvent thinned metallic ornamental paint consisting essentially of the following in parts by weight:

|                         |    |
|-------------------------|----|
| Asphalt                 | 7  |
| Coumarone-indene resin  | 7  |
| Mineral spirits         | 43 |
| Coal tar naptha solvent | 13 |
| Aluminum powder         | 10 |
| Asbestos fiber          | 20 |

5. A solvent thinned metallic ornamental paint consisting essentially of the following in parts by weight:

|                         |    |
|-------------------------|----|
| Asphalt                 | 9  |
| Coumarone-indene resin  | 6  |
| Mineral spirits         | 40 |
| Coal tar naptha solvent | 16 |
| Aluminum powder         | 12 |
| Asbestos fiber          | 17 |

6. A solvent thinned metallic ornamental paint consisting essentially of a binder of bituminous material selected from the group consisting of asphalt, coal tar pitches and stearine pitches, and coumarone-indene resin, in proportions of about 25% to 75% by weight of the bituminous material to about 75% to about 25% by weight of the resin; volatile solvent for the binder; aluminum powder; and a filler, the major proportion of which is asbestos fiber; the total quantity of binder and the solvent constituting about 67% to about 82% of the total weight of the paint; the

total quantity of the filler and the aluminum powder constituting about 18% to about 33% the total weight of the paint; the solvent to binder ratio being about 3 to 6 parts by weight of the solvent to about 1 part by weight of the binder; the filler to aluminum powder ratio being about 0.8 to 2.5 parts by weight of the filler to about 1 part by weight of the powder; the binder to aluminum powder ratio being about 1 to 2 parts by weight of the binder to about 1 part by weight of the aluminum powder; and the binder to the filler ratio being about 0.55 to 1.7 parts by weight of the binder to about 1 part by weight of the filler.

FREDERICK A. STOLZ,  
EDLEY J. VAUGHT, JR.

#### REFERENCES CITED

The following references are of record in the file of this patent:

#### UNITED STATES PATENTS

| Number       | Name         | Date          |
|--------------|--------------|---------------|
| 1,292,907    | Sperr et al. | Jan. 28, 1919 |
| 25 1,849,867 | Eckert       | Mar. 15, 1932 |
| 2,188,204    | Marc et al.  | Jan. 23, 1940 |
| 2,477,236    | Buchanan     | July 26, 1949 |

#### OTHER REFERENCES

"Asphalts and Allied Substances" by Abraham, 4th edition, page 55v, and Table 24 following page 370.